

1

3,171,737

## ELECTRICAL RESISTANCE ALLOY

Norman F. Spooner, Bloomfield Township, Oakland County, and Forbes S. Sibley, Birmingham, Mich., assignors to Hoskins Manufacturing Company, Detroit, Mich., a corporation of Michigan

No Drawing. Filed Apr. 28, 1961, Ser. No. 106,168  
6 Claims. (Cl. 75—124)

This invention relates to electrical resistance alloys and more particularly to an electrical resistance alloy having a relatively low temperature coefficient of resistivity and a moderate resistance.

The alloy is further characterized in that it can be drawn into extremely fine wire which is highly resistant to corrosion and the electrical properties of which are obtained without heat treatment after a conventional anneal.

The electrical resistant alloy of this invention is extremely useful in the manufacture of electrical apparatus which requires resistors of extremely high accuracy such as those used in radio, television, radar, etc. While resistors of this type do not have to be particularly resistant to oxidation at high temperature since they never heat to a temperature substantially beyond 150° C., it is very important that they possess relatively high resistance to atmospheric corrosion and relatively high strength. The strength requirements of these resistors arise from the fact that such resistors are in the form of extremely fine wire, for example, 40 gage wire (.003" diameter) and also wire having a diameter as small as .001" or less; and these fine wires must possess sufficient strength to withstand coiling by conventional methods. In addition, such high accuracy resistors, if they are to retain their accuracy for a long period of time, must be highly resistant to corrosion under atmospheric conditions.

Experience has shown that 30-gauge wires of this alloy, having about one hundred and thirty thousand p.s.i. tensile strength as annealed will produce fine wires of about .001" dia. which will have strength sufficient to allow winding of resistors by conventional methods. Specifications for such resistors usually require a temperature coefficient of resistivity (T.C.) of between  $\pm .000020$  ohm per ohm per ° C. in a temperature range of between -55° C. and 150° C. and a nominal resistivity of about 800 ohms per circular mil foot (c.m.f.).

Heretofore, alloys designed for use as such high accuracy resistors having the necessary strength and corrosion resistance have been of the nickel-chromium type. For example, one such alloy has a nominal composition of 20% chromium, 74% nickel, 3% aluminum, and 3% copper. Another such alloy has a nominal composition of 20% chromium, 2% to 4% aluminum, up to 6% iron, and the balance nickel.

The alloy of this invention, while having substantially the same electrical properties as the two previously mentioned alloys over the temperature range of -55° C. to 150° C., possesses distinct advantages thereover. The previously mentioned alloys have a very high nickel content, a critical and expensive material. In addition, the electrical properties referred to are developed in these alloys only after heat treatment. The alloy of this invention has a nominal composition of 5% aluminum, 4% molybdenum, 22% chromium, and the balance iron. Thus, in the alloy of the present invention, the nickel in the composition of the prior art alloys is replaced by iron; and furthermore, the present alloy possesses the desirable electrical properties without heat treatment. This latter feature is important in that by eliminating heat treatment, there is also eliminated slight variations in properties from one end of a spool of wire to the other because of slight non uniformities in temperature during heat treatment.

2

In addition, the alloy of this invention has a density approximately 10% less than the prior art alloys referred to which results in more feet of wire per pound. At the same time, by using molybdenum in the alloy in the range of 3% to 6%, the corrosion resistance and the strength of the alloy of this invention is equivalent to the two prior art alloys referred to. The alloy of this invention may have a nominal range of composition as follows: aluminum, 4.5% to 5.5%; chromium, 15.0% to 30.0%; molybdenum, 3.0% to 6.0%; silicon, 1.0% maximum; carbon, .1% maximum; iron, balance. The preferred range of composition of the present alloy is as follows: aluminum, 4.6% to 5.3%; chromium, 20.0% to 25.0%; molybdenum, 3.5% to 5.0%; silicon, 0.5% maximum; carbon, .08% maximum; iron, balance. Deoxidizers such as cerium, calcium, and zirconium may be present in the alloy in small amounts and are included in the above compositions in the iron content.

The presence of carbon in the alloy is due primarily to its presence in the iron and to its possible use in deoxidation. The silicon in the alloy results primarily from its presence in the chromium and the iron and also in its pick up from the crucible when a crucible formed of a silicon bearing ceramic, such as, zirconium silicate is employed. The presence of silicon may also result from the deoxidizing practice employed.

The aluminum range in the composition of the alloy has been determined on the basis of the following effects on the alloy:

- 30 (a) Its effect on the temperature coefficient of resistivity;
- (b) Its effect on resistivity; and
- (c) The effects of the melting practice on the aluminum requirement. For example, the amount of silicon pick up will affect the aluminum requirement.

The relationship between T.C. and resistivity varies somewhat with melting practice; but in general, an increasing aluminum content increases the resistivity and lowers the T.C. of the alloy. Alloys having a T.C. of  $\pm .000020$  will have a resistivity in the range of 780 to 860 ohms per c.m.f. For a given melting practice, the relationship between resistivity, T.C. and aluminum content follows the regular pattern stated; namely, an increasing aluminum content increases the resistivity and lowers the T.C.

The permissible range for the chromium content is rather broad because the properties of the alloy do not vary as much with chromium concentration as they do with aluminum. The range of the chromium content is determined by the T.C. and resistivity requirements and by the limited workability of alloys with higher chromium contents. In general, the chromium content of the alloy affects its properties in a manner similar to aluminum, but to a much lesser degree.

The molybdenum content of the alloy is based upon proper balance between:

- (a) The effect of molybdenum on strength;
- (b) The effect of molybdenum on corrosion resistance; and
- (c) The effect of molybdenum on workability.

The tensile strength of the alloy increases with an increase in molybdenum content to a maximum at about 3.5% to 4% molybdenum. An increase in the molybdenum content above 4% decreases the strength slightly. From the standpoint of strength alone, 3.5% to 4% molybdenum is optimum. With respect to corrosion resistance, this increases rapidly for the first .25% molybdenum and beyond that amount, increases at a decreasing rate as the molybdenum content is increased to about 5%. Beyond 5%

molybdenum, there is no substantial increase in the alloy's resistance to corrosion.

The molybdenum content of the alloy adversely affects its workability. However, with as much as 4% molybdenum, the alloy can be drawn to fine wire by normal processes; and at 6% molybdenum, the alloy can still be drawn, but with some difficulty. Above 6% molybdenum, the alloys cannot be drawn in accordance with conventional processes. Thus, the lower limit of the molybdenum in the composition is set at 3% molybdenum to provide adequate strength and corrosion resistance combined with a high degree of workability. The upper limit of molybdenum in the alloy is set at 5% to assure adequate strength and adequate workability. For extremely fine wire having a diameter of .003" or less, the upper limit of molybdenum in the alloy is set at 4% to enable adequate workability.

The preferred method of preparing the alloy comprises first melting high purity iron, chromium and molybdenum together at a reduced pressure in a suitable crucible, preferably magnesium oxide, to prevent pick up of secondary elements. After the oxygen content of the melt has been reduced by a suitable deoxidizing agent or agents, such as carbon, calcium, cerium or zirconium, high purity aluminum is added to the melt and allowed to mix with the alloy. The melt is then cast into suitable molds and ingots are worked to a final form such as wire by the normal process; that is, rolling and drawing. As is conventional, the wire is subjected to a final standard anneal to obtain the best temper for winding into resistors. The annealing can be done in a continuous manner at a temperature of between 1500° to 1800° F. in a non oxidizing atmosphere to preserve its bright finish.

It has been found that differences in the melting practice, such as the crucible material, the size of the heat, the type of deoxidizer and the type of atmosphere, can affect the properties of the alloy. For example, an alloy melted in air in a zirconium silicate crucible as a 480 lb. heat with calcium deoxidation, and having an aluminum content of 4.5%, had substantially the same T.C. and resistivity as a 46 lb. heat melted in vacuum in a zirconium silicate crucible with cerium deoxidation and having an aluminum content of 4.9%, the remainder of the composition being substantially the same for both alloys. As another example, one alloy containing 4.9% aluminum in a 46-pound ingot melted in the vacuum in a zirconium silicate crucible had substantially the same T.C. and resistivity as another alloy containing 5.3% aluminum in a 95-pound ingot melted in vacuum in a magnesium oxide crucible, the remainder of the composition being substantially the same for both alloys. The heat melted in zirconium silicate picked up silicon, which lowered the aluminum requirement. The ranges set forth above take into account the effects produced by different melting practices.

Below are set forth, in table form, a few examples of alloys of this invention and the properties of such alloys:

|        | Al  | Mo  | Cr   | Zr  | Si  | C   | T.M.<br>(-55/25° C.)<br>(p.p.m./° C.) | Annealed<br>Resis-<br>tivity,<br>ohms/<br>c.m.f. | Dia.<br>(in.) | Tensile<br>Strength<br>(p.s.i.) |
|--------|-----|-----|------|-----|-----|-----|---------------------------------------|--------------------------------------------------|---------------|---------------------------------|
| A----- | 4.7 | 4.0 | 22.0 | .15 | .5  | .03 | + 9                                   | 807                                              | .01           | 138,600                         |
| B----- | 5.3 | 3.9 | 21.0 | .33 | .02 | .03 | -10                                   | 831                                              | .01           | 140,000                         |
| C----- | 4.8 | 3.5 | 22.5 | .18 | .5  | .03 | -10                                   | 837                                              | .01           | 137,300                         |
| D----- | 4.6 | 3.8 | 22.5 | .18 | .5  | .03 | -19                                   | 832                                              | .01           | 142,300                         |
| E----- | 5.0 | 6.0 | 22.5 | .23 | .5  | .02 | -17                                   | 828                                              | .01           | 133,200                         |

Various melting practices were employed in these examples. However, they were all annealed in the same manner at approximately the same temperature.

This application is a continuation-in-part of our copending application Serial No. 801,722, filed March 25, 1959.

We claim:

1. A high strength, corrosion resistant electrical resistance element in the form of wire having a diameter of about .003" or less comprising an alloy producing without

heat treatment a temperature coefficient of resistivity of  $\pm .000020$  ohm per ohm per ° C. within the range of -55° C. to 150° C. and a resistivity of about 800 ohms per circular mil foot at 25° C., said alloy consisting essentially of 4.5% to 5.5% aluminum, 15% to 30% chromium, 3.0% to 4.0% molybdenum and the balance essentially iron.

2. A high strength, corrosion resistant electrical resistance element in the form of wire having a diameter of about .003" or less comprising an alloy producing without heat treatment a temperature coefficient of resistivity of  $\pm .000020$  ohm per ohm per ° C. within the range of -55° C. to 150° C. and a resistivity of about 800 ohms per circular mil foot at 25° C., said alloy consisting essentially of 4.6% to 5.3% aluminum, 20% to 25% chromium, 3.5% to 4.0% molybdenum and the balance essentially iron.

3. A high strength corrosion resistant electrical resistance element in the form of wire having a diameter of about .003" or less comprising an alloy producing without heat treatment a temperature coefficient of resistivity of  $\pm .000020$  ohm per ohm per ° C. within the range of -55° C. to 150° C. and a resistivity of about 800 ohms per circular mil foot at 25° C., said alloy consisting essentially of 4.5% to 5.5% aluminum, 15% to 30% chromium, 3.0% to 4.0% molybdenum, 1% maximum silicon, .1% maximum carbon, and the balance essentially iron.

4. A high strength corrosion resistant electrical resistance element in the form of wire having a diameter of about .003" or less comprising an alloy producing without heat treatment a temperature coefficient of resistivity of  $\pm .000020$  ohm per ohm per ° C. and a resistivity of about 800 ohms per circular mil foot at 25° C., said alloy consisting essentially of 4.6% to 5.3% aluminum, 20% to 25% chromium, 3.5% to 4.0% molybdenum, 1% maximum silicon, .1% maximum carbon, and the balance essentially iron.

5. A high strength corrosion resistant electrical resistance element in the form of wire having a diameter of about .003" or less comprising an alloy producing without heat treatment a temperature coefficient of resistivity of  $\pm .000020$  ohm per ohm per ° C. within the range of -55° C. to 150° C. and a resistivity of about 800 ohms per circular mil foot at 25° C., said alloy consisting essentially of about 5% aluminum, 4% molybdenum, 20% to 25% chromium and the balance essentially iron.

6. A high strength corrosion resistant electrical resistance element in the form of wire having a diameter of about .003" or less comprising an alloy producing without heat treatment a temperature coefficient of resistivity of  $\pm .000020$  ohm per ohm per ° C. within the range of -55° C. to 150° C. and a resistivity of about 800 ohms per circular mil foot at 25° C., said alloy consisting essentially of about 5% aluminum, 4% molybdenum, 20% to 25% chromium, 1% maximum silicon, .1% maximum carbon, and the balance essentially iron.

#### References Cited in the file of this patent

#### UNITED STATES PATENTS

70 1,833,723 Ruder ----- Nov. 24, 1931

#### FOREIGN PATENTS

680,930 Germany ----- Sept. 12, 1939  
617,194 Great Britain ----- Feb. 2, 1949